# EUROPEAN PATENT SPECIFICATION

(11) **EP 2 172 572 B1**
(45) Date of publication and mention of the grant of the patent: **15.05.2013**
(21) Application number: 08772999.2
(22) Date of filing: 30.06.2008
(51) Int. Cl.: C22C 21/02, C22C 21/00, C22F 1/043, C22F 1/04

(54) **A STRUCTURAL MATERIAL PART OF A HIGH-SI MG-CONTAINING AL ALLOY AND THE MANUFACTURE METHOD THEREOF**
BAUSTOFFTEIL AUS SI-REICHER MG-HALTIGER AL-LEGIERUNG UND HERSTELLUNGSVERFAHREN DAFÜR
PIÈCE DE MATÉRIAU DE STRUCTURE EN ALLIAGE D'AL CONTENANT MG ET À FORTE TENEUR EN SI ET PROCÉDÉ DE FABRICATION DE CELLE-CI

(30) Priority: 29.06.2007 CN 200710011919
(43) Date of publication of application: 07.04.2010
(73) Proprietor: Northeastern University, Heping District Shenyang Liaoning 110004 (CN)
(72) Inventor: ZUO, Liang, Liaoning 110004 (CN); YU, Fuxiao, Liaoning 110004 (CN); ZHAO, Gang, Liaoning 110004 (CN); ZHAO, Xiang, Liaoning 110004 (CN); YANG, Yongliang, Liaoning 110004 (CN); LI, Yan, Liaoning 110004 (CN)
(74) Representative: Vossius & Partner
(86) International application number: PCT/CN2008/001246
(87) International publication number: WO 2009/003365

(56) References cited:
- CN-A- 1 546 708
- CN-A- 1 555 423
- CN-A- 1 789 456
- GB-A- 582 732
- JP-A- 6 279 904
- JP-A- 01 017 834
- JP-A- 05 331 604
- JP-A- 08 003 701
- JP-A- 10 096 039
- JP-A- 62 083 453
- KR-A- 20000 041 707
- US-A- 4 068 645
- DATABASE WPI Week 200756 Thomson Scientific, London, GB; AN 2007-575922 XP002607664 -& JP 2007 118041 A (SHOWA DENKO KK) 17 May 2007 (2007-05-17)

## Description

### Background of the Present Invention

### Field of Invention

The present invention relates to aluminum alloys and their method of preparation, and more particularly to magnesium-contained high-silicon aluminum alloys for use as structural materials, and the manufacture method thereof.

### Description of Related Arts

Aluminum-silicon alloys (Al-Si alloys), especially those with high silicon content, are widely used in car and aviation industries, due to their low density, high wear resistance, high anti-corrosiveness, and low thermal expansion coefficient. With the common solidification method for preparation of Al-Si alloys, there usually appear large silicon particles and eutectic plates, resulting in a dramatically increased brittleness of the alloys. Thus, it is difficult to improve the solidified microstructure and to obtain various shaped high-performance structural materials through subsequent plastic deformation, which poses a bottleneck for more general applications of these alloys. Traditionally, Al-Si alloys are categorized into the casting aluminum alloy series. In order to overcome their poor deformation ability, some new processing methods based on rapid solidification or powder metallurgy have been explored. However, the rapid solidification method can only allow preparation of tiny ingots with a diameter less than 10mm. If a large-sized Al-Si alloy ingot is desired, a further process is then required. As for the powder metallurgy method, it enables to obtain a relatively large-sized part, but suffers from a complicated process with high fabrication cost.

In the existing methods for casting pure aluminum or aluminum alloys, the direct chill (DC) casting is most common in use. The main concerns are focused on how to reduce the chemical composition segregation, refine the solidification microstructure, and improve the ingot surface quality. Based on the DC casting route, an efficient manufacture method has been developed by one of the present inventers to prepare large-sized ingots of high silicon-containing aluminum alloys without adding any modifiers like P, Na, and Sr, and received a China Invention Patent with the patent number ZL200510119550.6. The present inventers have further found out that while narrowing the range of the Si content (i.e. increasing the lower limit to 8% by weight and reducing the upper limit to 18% by weight of Si concentration, and adjusting the contents of Mg the above method can be incorporated with thermoplastic processing and subsequent heat treatment, so as to produce Mg-containing high-silicon aluminum alloys with relatively high plasticity and strength, including profiles, bars, sheets, and forgings, for use as advanced new structural materials.

### Summary of the Present Invention

An object of the present invention is to provide high-silicon aluminum alloys (Al-Si alloys) that contain magnesium (Mg) and have good plasticity and high strength for use as structural materials, and the manufacture method thereof. Without adding any modifiers, the Al-Si alloys are manufactured at low cost with the direct chill casting followed by the thermoplastic process and heat treatment.

Accordingly, in order to accomplish the above object, the present invention presents the aluminum alloys containing Mg and high Si, which comprises profiles, bars sheets, and forgings, wherein the aluminum alloys are made by a process as defined in the claims, comprising the steps of:
(a) casting an alloy ingot by a method of direct chill casting;
(b) preheat-treating the ingot to disperse eutectic Si phase particles; and
(c) thermal-plastic processing and heat-treating to obtain the alloy with a final shape and a modified microstructure, wherein the strengthening mechanisms of the alloy are referred to the grain refinement strengthening of aluminum matrix, the dispersion strengthening of silicon particles, and the precipitation strengthening of second phase particles.

The Mg-contained high-silicon aluminum alloys for use as structural materials contains 0.2∼2.0wt% of Mg and 8∼18wt% of Si, wherein they have an evenly refined microstructure: the aluminum matrix is fine equiaxed with an average grain size less than 6µm, and the silicon and second phase particles are dispersed with an average size less than 5µm.

The Mg-contained high-silicon aluminum alloys may contain at least one of Cu, Zn, Ni, Ti, and Fe elements, wherein a total weight percentage of the Cu, Zn, Ni, Ti, and Fe is less than 2wt%.

The step (a) of direct chill casting is subjected to the cast ingot preparation for a given Al-Si alloy, at a relative casting temperature of 150∼300°C above the liquidus line, a casting speed of 100∼200mm/min, and a cooling water flux of 5∼15g/mm·s on the periphery of the solidified ingot, wherein no modifier is added to the alloy.

The step (b) of preheat-treating is subjected to the formation of dispersed eutectic Si phase particles in the ingot, at a heating rate of 10∼30°C/min, a heating temperature of 450∼520°C, and a holding time of 1∼3 hours.

The preheat-treated ingot is subjected to a thermal-plastic processing in the step (c), at a hot-deformation temperature of 400∼520°C, followed by cooling naturally or forcedly. The hot-deformed product is then heat-treated after the thermal-plastic processing.

For the product thermal-plastic processed with natural cooling, the heat treatment in the step (c) further comprises a step of solution treatment and a step of artificial aging process. The solution treatment is performed at a heating rate of 10∼30°C/min, a solution treatment temperature of 500∼540°C, and a solution treatment time of 0.5~3 hours, followed by quenching. The artificial aging process is performed at an aging temperature of 160∼200°C, and an aging time of 1∼10 hours.

For the product thermal-plastic processed with forced cooling, the heat treatment in the step (c) further comprises a step of artificial or natural aging treatment, wherein the artificial treatment is performed at an aging temperature of 160∼200°C, and an aging time of 1∼10 hours.

A hot rolling process is adapted in the step of thermal-plastic processing, wherein the ingot is hot deformed at a total rolling reduction of more than 40%.

A hot extrusion process is adapted in the step of thermal-plastic processing, wherein the ingot is hot deformed at an extrusion ratio of more than 15.

A hot forging process is adapted in the step of thermal-plastic processing, wherein the ingot is hot deformed at a forging ratio of more than 40%.

The present invention overcomes the cognition prejudice traditionally imposed on Al-Si alloys. Without adding any modifiers, an unexpected effect has been reached on the magnesium-contained high-silicon aluminum alloys prepared by incorporating conventional direct chill casting method with thermal-plastic process and heat treatment. They are typically of fine-dispersed silicon particles and second phase at equiaxed Al matrix, associated with a relatively high strength and good plasticity for potential use as structural materials

Fig. 14 gives a comparison of mechanical properties between the Al-Si extrusion alloys of the present invention and the China National Standard extrusion alloy 6063 at the T5 and T6 states, wherein the alloys of the present invention are AI-8.5Si-1.8Mg-0.27Fe, Al-12.7Si-0.7Mg-1.5Cu-0.3Ni-0.3Ti-0.3Fe, and Al-15.5Si-0.7Mg-0.27Fe, respectively.

Notably, the yield strength and tensile strength of the Al-8.5Si-1.8Mg-0.27Fe, Al-12.7Si-0.7Mg-1.5Cu-0.3Ni-0.3Ti-0.3Fe, and Al-15.5Si-0.7Mg-0.27Fe extrusion alloys at the T6 state are higher than the China National Standards for the extrusion alloy 6063 at the T6 state. The mechanical properties of these alloys at the extrusion state (T1), especially the elongation rate, are also higher than the China National Standards for the 6063 alloys at the T5 state.

As the most common aluminum extrusion alloys, the 6063 alloys have been widely used in architectures, vehicles, and decorations etc., which have great need in the existing market. Once the 6063 alloys are partially replaced by the magnesium-contained high-silicon aluminum alloys of the present invention, it will bring great economic benefits. In addition, the use of an increased amount of Si in the alloys can dramatically conserve the aluminum resource.

These and other objectives, features, and advantages of the present invention will become apparent from the following detailed descriptions, the accompanying drawings, and the appended claims.

### Brief Description of the Drawings

FIG. 1 is a perspective view of a device of direct chill casting according to preferred embodiments of the present invention.
FIG. 2 is a microstructure of ingot of Al-12.7Si-0.7Mg-0.3Fe alloy (#3) at cast condition during the direct chill casting process according to the present invention, wherein a casting temperature is 730°C, a casting rate is 180mm/min, and a cooling water flow rate is 8g/mm·s.
FIG. 3 is a high magnification microstructure of ingot of Al-12.7Si-0.7Mg-0.3Fe alloy (#3) at cast condition during the direct chill casting process according to the present invention, wherein a casting temperature is 730°C, a casting rate is 180mm/min, and a cooling flow rate of the surrounding water is 8g/mm·s.
FIG. 4 is a microstructure of Al-12.7Si-0.7Mg-0.3Fe alloy (#3) after pre-heated to 500°C for 2 hours, heat extruded at 470°C (having extrusion ratio of 15) according to the present invention.
FIG. 5 is a T6 state microstructure of Al-12.7Si-0,7Mg-0.3Fe alloy (#3) after pre-heated to 500°C for 2 hours, heat extruded at 470°C (having extrusion ratio of 15) according to the present invention, wherein said T6 state is at a solution temperature 540°C for one hour, and at an artificial aging temperature 200°C for 3 hours.
FIG. 6 is a microstructure of ingot of Al-15.5Si-0.7Mg-0.27Fe alloy (#5) at cast condition during the direct chill casting process according to the present invention, wherein the casting temperature is 800°C, a casting rate is 140 mm/min, and the cooling water flow rate is 10g/mm·s.
FIG. 7 is a high magnification microstructure of ingot of Al-15.5Si-0.7Mg-0.27Fe alloy (#5) at cast condition during the direct chill casting process according to the first preferred embodiment of the present invention, wherein the casting temperature is 800°C, the casting rate is 140mm/min, and the cooling water flow rate is 10g/mm·s.
FIG. 8 is a microstructure of Al-15.5Si-0.7Mg-0.27Fe alloy (#5) after pre-heated to 500°C for 2 hours, heat extruded at 470°C (having extrusion ratio of 45) according to the present invention.
FIG. 9 is a microstructure of Al-15.5Si-0.7Mg-0.27Fe alloy (#5) after pre-heated to 500°C for 1 hour, heat rolled at 500°C (pressing amount of 60%) according to the present invention.
FIG. 10 is a T6 state microstructure of ingot of Al-15.5Si-0.7Mg-0.27Fe alloy (#5) after pre-heated to 500°C for 2 hours, heat extruded at 470°C (having extrusion ratio of 45) according to the present invention, wherein said T6 state is at a solution temperature 520°C for 2 hours, and at an artificial aging temperature 180°C for 4 hours.
FIG. 11 is a T6 state microstructure of rectangular ingot of Al-15.5Si-0.7Mg-0.27Fe alloy (#5) after pre-heated to 500°C for 1 hour, heat rolling at 500°C (pressing amount of 60%) according to the present invention, wherein said T6 state is at a solution temperature 520°C for 3 hours, and at an artificial aging temperature 200°C for 4 hours.
FIG. 12 is a T6 state of high rate microstructure of Al-15.5Si-0.7Mg-0.27Fe alloy (#5) after pre-heated to 500°C for 2 hours, heat extruded at 470°C (having extrusion ratio of 45) according to the present invention, wherein said T6 state is at a solution temperature 520°C for 2 hours, and at an artificial aging temperature 180°C for 4 hours.
FIG. 13 is a microstructure of ingot of Al-17.5Si-0.7Mg-1.0Cu-0.27Fe alloy (#7) at cast condition during the direct chill casting process according to the present invention, wherein the casting temperature is 850°C, a casting rate is 120mm/min, and the cooling water flow rate is 10/mm·s.
FIG. 14 is a table showing the comparisons mechanical properties of extrusion Si Al alloy of the present invention and the China standard extrusion of 6063 alloy.
FIG. 15 is a table showing the compositions of an alloy made from the ingot via the casting process.
FIG. 16 is a table showing the parameters of different alloys through casting process.
FIG. 17 is a table showing the parameters of the pre-heating process and extrusion process of each of alloys.
FIG. 18 is a table showing the parameters of the pre-heating process and rolling process of each of alloys.
FIG. 19 is a table showing the parameters of the pre-heating process and forging process of each of alloys.
FIG. 20 is a table showing the parameters of the extrusion process for different alloys.
FIG. 21 is a table showing the parameters of the rolling process for different alloys.
FIG. 22 is a table showing the parameters of the forging process for different alloys.
FIG. 23 is a table showing the mechanical properties under variety of deformation processes and heat treatments situations.

### Detailed Description of the Preferred Embodiment

Referring to Fig. 1 of the drawings, a step of casting ingot via the direct chill casting method according to the present invention is illustrated.

A device designed for the direct chill casting process is shown in Fig. 1 of the drawings, wherein the device comprises a cooling water inlet 1, a crystallizer 2, a hot top 4, and a graphite ring 5, wherein a raw material 3 of the ingot and a liquid metal 6 are separately received within a container of the device. A plurality of compositions of an alloy made from the ingot via the casting process is shown in Fig. 15. A plurality of parameters of the casting process is shown in Fig. 16.

Referring to Figs. 17, 18, and 19, a step of preheating, followed by hot extruding, or hot rolling, or hot forging the ingot according to the present invention is illustrated.

In the preheating process, the ingot is heated in an oven at a predetermined heating rate. After the predetermined temperature is reached, the ingot is held for a predetermined time. Then, a hot extrusion device, or a hot rolling device, or a hot forging device is used to complete a thermal-plastic processing. A plurality of parameters of the preheating and hot extruding for each of the alloys is shown in Fig. 17. A plurality of parameters of the preheating and hot rolling for each of the alloys is shown in Fig. 18. A plurality of parameters of the preheating and hot forging for each of the alloys is shown in Fig. 19.

Referring to Figs. 20, 21, 22, and 23, a step of heat treatment after hot deformation of the alloys, such as hot extrusion, hot rolling, and hot forging, according to the present invention is illustrated.

After the hot extrusion, hot rolling, or hot forging process of the ingot, the heat treatment is applied to the product at a predetermined temperature. A plurality of parameters of the hot extrusion, hot rolling, and hot forging processes are shown in Figs. 20, 21, and 22 respectively. A plurality of mechanical properties of the alloys after the heat treatments is shown in Fig. 23.

The present invention provides the industrial use of the Mg-contained high silicon aluminum alloys (Al-Si alloy), and the manufacture method thereof. Without adding any modifiers, the Al-Si alloys having good plasticity and relatively high strength are manufactured at low cost with the direct chill casting followed by the thermal-plastic process and heat treatment, for use as structural materials.

One skilled in the art will understand that the embodiment of the present invention as shown in the drawings and described above is exemplary only and not intended to be limiting.

It will thus be seen that the objects of the present invention have been fully and effectively accomplished. The embodiments have been shown and described for the purposes of illustrating the functional and structural principles of the present invention and is subject to change without departure from such principles. Therefore, this invention includes all modifications encompassed within the scope of the following claims.

## Claims

1. A process for manufacturing aluminum alloy product containing 0.2~2.0 weight percentage (wt%) of Mg, 8∼18wt% of Si and having an evenly refined microstructure, an equiaxed aluminum matrix with an average grain size < 6µm, and silicon and second phase particles dispersed with an average size < 5µm, such as sectional material, bar, sheet, and forging, comprising the steps of:
(a) casting an ingot of said aluminum alloys by direct chill casting; wherein said direct chill casting is performed at a relative casting temperature of 150∼300°C above the liquidus line of said aluminum alloys, a casting speed of 100∼200mm/min, and a cooling water flux of 5∼15g/mm·s on the periphery of said ingot, wherein no modifier is added in said direct chill casting;
(b) preheat-treating said ingot to disperse eutectic Si phase particles at a heating rate of 10∼30°C/min, a heating temperature of 450∼520°C, and a holding time of 1∼3 hours; and
(c) thermal-plastic processing then coding and then heat-treating to obtain said aluminum alloy product with a final shape and a modified microstructure, wherein the strengthening mechanisms of said aluminum alloys are grain refinement strengthening of the aluminum matrix, dispersion strengthening by silicon particles, and precipitation strengthening of second phase particles,
wherein said aluminum alloy is cooled naturally or is cooled forcedly, and it is heat-treated after said thermal-plastic processing.

2. The process, according to claim 1, wherein said alloy of said structural material contains at least one of Cu, Zn, Ni, Ti, and Fe, wherein a total weight percentage of said Cu, Zn, Ni, Ti, and Fe is equal or less than 2wt%.

3. The process according to claim 1 or 2 wherein the step (c) step of solution treatment and a step of artificial aging treatment consists of a natural cooling after the thermal-plastic processing followed by a , wherein said solution treatment is performed at a heating rate of 10∼30°C/min, a solution treatment temperature of 500∼540°C, and a solution treatment time of 0.5∼3 hours followed by quenching and said artificial aging treatment is performed at an aging temperature of 160∼200°C, and an aging time of 1∼10 hours.

4. The process according to claim 1 or 2 wherein the step (c) step of artificial or natural aging treatment consists of a forced cooling after the thermal-plastic processing followed by a and if the aging is artificial aging, it is performed at an aging temperature of 160∼200°C, and an aging time of 1∼10 hours.

5. The process according to claim 1 or 2 wherein the step (c) further comprises a step of hot rolling in said thermal-plastic processing, wherein the total reduction amount or said hot rolling is greater than 40%.

6. The process according to claim 1 or 2 wherein the step (c) further comprises a step of hot extrusion in said thermal-plastic processing, wherein the extrusion ratio of said hot extrusion is greater than 15.

7. The process according to claim 1 or 2 wherein the step (c) further comprises a step of hot forging in said thermal-plastic processing, wherein the forging ratio of said hot forging is greater than 40%.

## Patentansprüche

1. Verfahren zum Herstellen eines Aluminiumlegierungsprodukts das 0,2-2,0 Gewichtsprozent (Gew.-%) Mg, 8~18 Gew.-% Si enthält und eine gleichmäßig feine Mikrostruktur, eine gleichachsige Aluminiummatrix mit einer durchschnittlichen Korngröße <6 µm, und Teilchen aus Silizium und einer zweiten Phase aufweist, die mit einer durchschnittliche Größe <5 µm dispergiert sind, wie ein Profilmaterial, Stab, Blech und Schmiedestück, das die Schritte aufweist:
(a) Gießen eines Blocks der Aluminiumlegierungen durch direktes Kokillengießen (direct chill casting), wobei das direkte Kokillengießen bei einer relativen Gießtemperatur von 150∼300°C über der Liquiduslinie der Aluminiumlegierungen, einer Gießgeschwindigkeit von 100~200 mm/min und einem Kühlwasserfluss von 5~15 g/mm·s auf den Umfang des Blocks durchgeführt wird, wobei kein Modifiziermittel beim direkten Kokillengießen hinzugefügt wird;
(b) Vorerwärmungsbehandeln des Blocks, um Teilchen einer eutektischen Si-Phase zu dispergieren, mit einer Erwärmungsgeschwindigkeit von 10∼30°C/min, einer Erwärmungstemperatur von 450∼520°C und einer Haltezeit von 1~3 Stunden;
und
(c) thermoplastisches Bearbeiten, dann Abkühlen und dann Wärmebehandeln, um das Aluminiumlegierungsprodukt mit einer endgültigen Form und einer modifizierten Mikrostruktur zu erhalten, wobei die Festigkeitserhöhungsmechanismen der Aluminiumlegierungen Kornverfeinerungsfestigkeitserhöhung der Aluminiummatrix, Dispersionsfestigkeitserhöhung durch Siliziumteilchen und eine Ausscheidungsfestigkeitserhöhung der Teilchen der zweiten Phase sind, wobei die Aluminiumlegierung selbstgekühlt oder zwangsgekühlt wird, und nach dem thermoplastischen Bearbeiten wärmebehandelt wird.

2. Verfahren nach Anspruch 1, wobei die Legierung des Baumaterials mindestens eines von Cu, Zn, Ni, Ti und Fe enthält, wobei ein Gesamtgewichtsanteil des Cu, Zn, Ni, Ti und Fe gleich oder kleiner 2 Gew.-% ist.

3. Verfahren nach Anspruch 1 oder 2, wobei der Schritt (c) aus Selbstkühlen nach dem thermoplastischen Bearbeiten gefolgt von einem Schritt einer Lösungsbehandlung und einem Schritt einer künstlichen Alterungsbehandlung besteht, wobei die Lösungsbehandlung mit einer Erwärmungsgeschwindigkeit von 10∼30°C/min, einer Lösungsbehandlungstemperatur von 500∼540°C und einer Lösungsbehandlungszeit von 0,5∼3 Stunden gefolgt von Abschrecken durchgeführt wird, und die künstliche Alterungsbehandlung bei einer Alterungstemperatur von 160∼200°C und einer Alterungszeit von 1~10 Stunden durchgeführt wird.

4. Verfahren nach Anspruch 1 oder 2, wobei der Schritt (c) aus einem Zwangsabkühlen nach dem thermoplastischen Bearbeiten gefolgt von einem Schritt einer künstlichen oder natürlichen Alterungsbehandlung besteht, und wenn die Alterung eine künstliche Alterung ist, sie mit einer Alterungstemperatur von 160∼200°C und einer Alterungszeit von 1~10 Stunden durchgeführt wird.

5. Verfahren nach Anspruch 1 oder 2, wobei der Schritt (c) ferner einen Schritt des Warmwalzens im thermoplastischen Bearbeiten aufweist, wobei der Gesamtreduzierungsbetrag des Warmwalzens größer als 40% ist.

6. Verfahren nach Anspruch 1 oder 2, wobei der Schritt (c) ferner einen Schritt des Warmstrangpressens im thermoplastischen Bearbeiten aufweist, wobei das Strangpressverhältnis des Warmstrangpressens größer als 15 ist.

7. Verfahren nach Anspruch 1 oder 2, wobei der Schritt (c) ferner einen Schritt des Warmschmiedens im thermoplastischen Bearbeiten aufweist, wobei das Schmiedeverhältnis des Warmschmiedens größer als 40% ist.

## Revendications

1. Procédé de fabrication d'un produit d'alliage d'aluminium contenant de 0,2 à 2,0 pour cent en poids (% pds) de Mg, 8 à 18 % pds de Si et présentant une microstructure de finesse homogène, une matrice aluminium équiaxe avec une granularité moyenne < 6 µm, et des particules de silicium et de phase secondaire dispersées avec une granulométrie moyenne < 5 µm, tel qu'un matériau profilé, une barre, une feuille ou une pièce forgée, comprenant les étapes suivantes :
(a) moulage d'un lingot de l'alliage d'aluminium par procédé de moulage direct en coquille, ledit moulage direct en coquille étant exécuté avec une température relative de coulée comprise entre 150 et 300°C au-dessus de la ligne du liquidus de l'alliage d'aluminium, une vitesse de coulée comprise entre 100 et 200 mm/min, et un débit d'eau de refroidissement compris entre 5 et 15 g/mm·s à la périphérie du lingot, aucun élément modificateur n'étant ajouté à la coulée de moulage direct en coquille ;
(b) traitement par préchauffage du lingot pour disperser les particules de phase Si eutectique avec une vitesse de chauffage comprise entre 10 et 30°C/min, une température de chauffage comprise entre 450 et 520°C, et un temps de maintien compris entre 1 et 3 heures ; et
(c) traitement thermoplastique, suivi d'un refroidissement, lui-même suivi d'un traitement thermique afin d'obtenir le produit d'alliage d'aluminium avec une forme définitive et une microstructure modifiée, les mécanismes de renforcement de l'alliage d'aluminium étant un renforcement par affinage de grain de la matrice aluminium, renforcement par dispersion des particules de silicium, et renforcement par précipitation des particules de phase secondaire, l'alliage d'aluminium étant refroidi naturellement ou subissant un refroidissement forcé, et étant soumis à un traitement thermique consécutif au traitement thermoplastique.

2. Procédé selon la revendication 1, où l'alliage du matériau de structure contient au moins un des éléments suivants : Cu, Zn, Ni, Ti, et Fe, un pourcentage en poids total de Cu, Zn, Ni, Ti, et Fe étant inférieur ou égal à 2 % pds.

3. Procédé selon la revendication 1 ou la revendication 2, où l'étape (c) consiste en un refroidissement naturel consécutif au traitement thermoplastique, suivi par une étape de traitement de mise en solution et une étape de traitement par vieillissement artificiel, le traitement de mise en solution étant exécuté avec une vitesse de chauffage comprise entre 10 et 30°C/min, une température de traitement de mise en solution comprise entre 500 et 540°C, et un temps de traitement de mise en solution compris entre 0,5 et 3 heures, suivie d'une trempe, et le traitement par vieillissement artificiel étant exécuté avec une température de vieillissement comprise entre 160 et 200°C, et un temps de vieillissement compris entre 1 et 10 heures.

4. Procédé selon la revendication 1 ou la revendication 2, où l'étape (c) consiste en un refroidissement forcé consécutif au traitement thermoplastique, suivi par une étape de traitement par vieillissement artificiel ou naturel et où, si le vieillissement est un vieillissement artificiel, celui-ci exécuté avec une température de vieillissement comprise entre 160 et 200°C, et un temps de vieillissement compris entre 1 et 10 heures.

5. Procédé selon la revendication 1 ou la revendication 2, où l'étape (c) comprend en outre une étape de laminage à chaud lors du traitement thermoplastique, la valeur de réduction totale du laminage à chaud étant supérieure à 40 %.

6. Procédé selon la revendication 1 ou la revendication 2, où l'étape (c) comprend en outre une étape d'extrusion à chaud lors du traitement thermoplastique, le taux d'extrusion de l'extrusion à chaud étant supérieur à 15.

7. Procédé selon la revendication 1 ou la revendication 2, où l'étape (c) comprend en outre une étape de forgeage à chaud lors du traitement thermoplastique, le taux de forgeage à chaud étant supérieur à 40 %.
